

# UNITED STATES PATENT OFFICE.

GEORG BURGSCHMIET, OF MORDEN, MANITOBA, CANADA.

## EXPLOSIVE.

1,139,339.

Specification of Letters Patent.

Patented May 11, 1915.

No Drawing.

Application filed January 12, 1914. Serial No. 811,753.

To all whom it may concern:

Be it known that I, GEORG BURGSCHMIET, a citizen of the German Empire, and a resident of Morden, Province of Manitoba, Dominion of Canada, have invented certain new and useful Improvements in Explosives, of which the following is a specification.

This invention has reference to a new and improved explosive of that type which is not easily subject to spontaneous explosion and therefore may be safely transported and stored. The novel explosive comprises essentially nitrate of ammonium or ammonia 10 saltspeter as it is commonly called.

It has been well known for a long time that nitrate of ammonium is decomposed by heat forming nitrous oxid and water vapor and when the nitrous oxid is slightly over-heated decomposition accompanied by explosion takes place. It is apparent from the constitution of the nitrate of ammonium that not alone spontaneous explosions are prevented, but that no poisonous gases are 20 formed. It has been the aim to utilize nitrate of ammonium for explosives which may be safely transported and stored without being subject to spontaneous explosion such as may happen with dynamite, nitro-glycerin and the like. This has been primarily attained in the present invention by compounding the nitrate of ammonium with certain di- tri and tetranitro compounds of the aromatic series containing one or two 30 benzene rings or nuclei in the molecule such as, for instance, di- and tri-nitrotoluenes or di- tri or tetranitronaphthalenes. Further, some dry vegetable substances are incorporated which act as retarding elements and 35 serve for the propagation of the ignition.

The principal components of the present explosive clearly show that it withstands atmospheric influences and is not affected by moderate heat, cold or moisture. Likewise 45 shocks, blows or a fall such as occur during transportation or incidentally will not affect the explosive. Furthermore, comparative tests have shown that the novel explosive is more desirable than other explosives pertaining to the class of the so-called "safety explosives" and its manufacture is considerably more simple and cheap.

In carrying the invention into effect the nitrate of ammonium  $\text{NH}_4\text{NO}_3$  is pulverized. The nitro compound of the aromatic 55 series is then reduced and both substances

are thoroughly mixed together with a small percentage of powdered charcoal and a slight percentage of wood meal.

The process of preparing the explosive 60 thus is very simple and free from danger and accidents as long as the mixing is carried out at ordinary temperature. It is, of course, necessary that the substances, when being mixed, be dry and the final product 65 must also be kept in a dry condition.

The proportions in which the above enumerated components are compounded are substantially as follows:

|                                                                                   |      |    |
|-----------------------------------------------------------------------------------|------|----|
| Nitrate of ammonium about                                                         | 80%  | 70 |
| Dinitrotoluene $\text{C}_6\text{H}_3\text{CH}_3\text{(NO}_2\text{)}_2$ ,<br>about | 18%  |    |
| Charcoal and wood meal about                                                      | 2%   |    |
| Total                                                                             | 100% | 75 |

For certain applications the percentages of the various components may be varied. Likewise, a change in the percentages may be made when certain nitro compounds of 80 the aromatic series are used. For instance, the tetranitronaphthalene  $\text{C}_{10}\text{H}_4\text{(NO}_2\text{)}_4$  explodes violently when quickly heated and therefore less, say only 15%, is used, while in this instance the percentage of nitrate of 85 ammonium is correspondingly increased. If a dinitro product is used then a higher percentage is desirable and accordingly the nitrate of ammonium may be reduced as far down as 70%. The charcoal and wood meal 90 may also be varied from 0.5 to 2%. If a quick initiation and propagation of the ignition is desired, a little more charcoal is added and vice versa.

The proportions of the ingredients herein-before stated produce an explosive for rather general application. However, the stated variations are desirable according to the nature of the different kinds of rocks and deposits in quarries and mines which 100 are different and therefore require a somewhat modified explosive. Sometimes it is required to blast a rock to pieces in a rather destructive manner and in other cases blocks of rock should be merely separated and 105 moved forward without any destructive effect, so that the separated blocks may be split into plates like slabs of marble. In the first instance, a high explosive effect is necessary and in the second a rather retarded and slower effect is desirable. Variations in the percentages of the different compo-

ments within reasonable limits, the selection of the proper nitro compound of the aromatic series, and the mode of application render the novel explosive useful under the 5 described different conditions and requirements.

I claim as my invention:

An explosive comprising essentially about 80% of nitrate of ammonium, about 18% of

dinitrotoluene, and about 2% of charcoal 10 and wood meal.

Signed at Morden this 5th day of January, 1914.

GEORG BURGSCHMIET.

Witnesses:

J. B. WEBER,  
CLIFFORD WEIR.